

R. T. JOHNSTON.  
METHOD OF CASTING PRINTING PLATES.  
APPLICATION FILED OCT. 21, 1912.

1,092,487.

Patented Apr. 7, 1914.



Witnesses:

G. J. Donarosko Jr.  
A. Burkhardt

Inventor:

Robert T. Johnston,  
by Adams of Jackson.

Atty's

# UNITED STATES PATENT OFFICE.

ROBERT T. JOHNSTON, OF CHICAGO, ILLINOIS, ASSIGNOR TO THE GOSS PRINTING PRESS COMPANY, OF CHICAGO, ILLINOIS, A CORPORATION OF ILLINOIS.

## METHOD OF CASTING PRINTING-PLATES.

1,092,487.

Specification of Letters Patent.

Patented Apr. 7, 1914.

Application filed October 21, 1912. Serial No. 726,976.

*To all whom it may concern.*

Be it known that I, ROBERT T. JOHNSTON, a citizen of the United States, residing at Chicago, in the county of Cook and State 5 of Illinois, have invented a certain new and useful Method of Casting Printing-Plates, of which the following is a specification, reference being had to the accompanying drawing.

10 This invention relates to a new and improved method of casting printing plates and apparatus therefor.

Many processes differing more or less from each other have been employed for 15 producing printing plates. By some processes the plate is cast entire in an appropriate mold, either cast curved for use in that condition or cast flat for use on a flat-bed press or to be curved by a subsequent op-

20 eration for use on a cylinder press. By other processes, a metal printing face is produced in the form of a shell, which shell it is necessary by a subsequent operation to back up properly to strengthen it for use.

25 A much-used method of backing up such a shell comprises the placing of the shell in position in a casting-box so that the shell itself forms the front face of the plate, the rear face of which is defined by the back 30 of the casting-box or mold.

In most cases it is highly important to cool the finished printing plate as rapidly as is consistent with good workmanship. However, it has always been found necessary 35 to cool the printing face of a cast plate gradually up to a certain well-recognized limit in order to prevent a distortion of the figures upon the plate such as to render the plate imperfect or even useless. It has there-

40 fore been the practice to protect the face of the plate against rapid cooling, while at the same time the back of the plate has been cooled much more rapidly. To this end, the back of the casting box or mold has been 45

formed of metal, usually iron, and steps have been taken to bring about a rapid cooling of the back of the casting box, very often by the expedient of forcing water into contact with the back of the casting box.

50 The result of this has been that the back of the plate so chilled has had a mottled appearance and has shrunk irregularly so as to produce a varied thickness through the plate. To counteract this irregularity in 55 thickness, in order that the plate might be

of the required thickness so as to bring the printing face of the plate precisely at the desired point when the plate is applied to a press, it has been customary to provide the back of the plate in casting with a plurality of ribs by reason of which the effective thickness of the plate has been made slightly greater than the desired thickness. Then by a subsequent operation the ribs have been planed or shaved off to bring the effective 60 thickness of the plate to precisely the dimensions desired. 65

It is the object of this invention to improve the processes of producing printing plates in such a manner as to insure that 70 the plate shall be of the desired effective thickness as originally cast and so render the planing or shaving of the back of the plate or of the ribs thereof unnecessary.

It is a further object of this invention to 75 provide means by the use of which a plate may be cast of the desired effective thickness without the necessity for the shaving operation.

I have accomplished the objects I seek 80 by the expedient of protecting the faces of the ribs of the newly-cast plate so that they are not permitted to cool so rapidly as to render them uneven and unreliable. This I accomplish by cutting the grooves in the 85 back of the casting-box or mold considerably deeper than is necessary for the formation of the ribs on the back of the plate, and by providing each of such grooves with a member composed of material which is a 90 very poor conductor of heat, the poor heat-conducting member of course being proportioned so as to secure the desired aggregate thickness of the plate and the ribs thereon.

The particular embodiment of the apparatus by which I have accomplished these objects is illustrated in the drawings and hereinafter specifically described.

That which I believe to be new is set forth in the claims.

The drawing is a cross sectional view of the back of a casting-box and a printing plate in position thereagainst, partly broken away, the same being an embodiment of the preferred form of my invention.

In this drawing, 10 indicates a metal plate forming the back of a casting-box, provided with heat-radiating ribs 11 on its outer face. 105 12 indicates a plurality of grooves in the inner face of said plate 10, said grooves be- 110

ing almost completely filled by the blocks of poor heat-conducting material 13.

14 indicates a printing plate, the upper printing face of which is produced in any 5 suitable manner.

15 indicates the ribs formed on the back of the printing plate 14 against the faces of the poor heat-conducting members 13.

As will be readily understood, when the 10 molten printing plate metal is poured into the casting-box, that portion of the molten metal which comes in contact with the metal plate 10 will be readily cooled by reason of the fact that such plate 10 is a very good 15 conductor of heat. But the faces of the ribs 15 cannot be so readily cooled by reason of the fact that the members 13 are poor conductors of heat. It therefore follows that, while the printing plate 14 as a whole can be 20 cooled almost as rapidly as though the members 13 were not employed, the cooling of the faces of the ribs 15 is very materially retarded and rapid cooling of such faces is prevented. The result is that the ribs 15 do 25 not become "cold-shot", or "chilled", or mottled in appearance, in the manner above described which is objectionable for the reasons above stated, but the cooling is caused to proceed more slowly at such a rate that 30 the metal shrinks evenly. In case the members 13 are all located and proportioned so that their faces are at the same distance from the printing face of the plate produced, it follows that the aggregate thickness 35 of the printing plate 14 and the ribs 15 is uniform throughout the plate 14, and in case the proportions are such as to produce a plate 14 the effective thickness of which,—that is to say, the aggregate thickness of the 40 plate proper and of the ribs,—conforms to the thickness of plate desired for use on a press, then it follows that there is no need for shaving the ribs of the printing plate after it is removed from the casting-box.

45 By reason of this invention, doing away with the necessity for shaving the ribs of the plates produced, a very material saving of time in the preparation of a plate is effected, which, as said above, is of very great 50 importance, especially in the preparation of the plates for the run of a daily newspaper.

While I have shown the preferred form of device for practising the method above set forth, it will be understood that I do not

wish to restrict myself to the form shown 55 except as hereinafter specifically claimed. So far as I am aware, it is new in the art to protect the part of the cast plate which is to serve as a bearing for the plate upon a press against rapid cooling, and my claims 60 are to be construed accordingly.

What I claim as my invention and desire to secure by Letters Patent is,—

1. The method of casting a printing plate, which comprises retarding the cooling of the 65 portion of the plate which forms a bearing for the plate upon a press.

2. The method of casting a printing plate, which comprises protecting the portion of the plate which forms a bearing for the 70 plate upon a press against rapid cooling.

3. The method of casting a printing plate, which comprises cooling the major portion of the back face of the plate and retarding the cooling of the portion of the plate which 75 forms a bearing for the plate upon a press.

4. The method of casting a printing plate, a portion only of the back face of which forms the bearing for the plate upon a press, which comprises cooling the back face 80 of said plate with the exception of said bearing portion and retarding the cooling of said bearing portion.

5. The method of casting a printing plate having projecting portions on its back face 85 which form the bearing for the plate upon a press, which comprises retarding the cooling of the bearing faces of said projecting portions and cooling the remainder of the back of said plate.

6. The method of casting a printing plate having ribs on its back face, which comprises retarding the cooling of said ribs.

7. The method of casting a printing plate having ribs on its back face, which comprises protecting the faces of said ribs 95 against rapid cooling.

8. The method of casting a printing plate having ribs on its back face, which comprises protecting the faces of said ribs 100 against rapid cooling and at the same time cooling the remainder of the back face of said plate.

ROBERT T. JOHNSTON.

Witnesses:

W. H. DE BUSK,  
W. A. FURNNER.